

# United States Patent Office.

OLIVER T. MAY, OF CANASTOTA, NEW YORK.

*Letters Patent No. 99,216, dated January 25, 1870.*

## IMPROVED NON-CORROSIVE METALLIC ROOFING.

The Schedule referred to in these Letters Patent and making part of the same.

To all whom it may concern:

Be it known that I, OLIVER T. MAY, of Canastota, in the county of Madison, and in the State of New York, have invented a new and improved Non-Corrosive Metallic Roofing; and I do hereby declare that the following is a full, clear, and exact description thereof.

The nature of my invention consists in the combination of tin, copper, and lead in certain proportions, to form a non-corrosive alloy for roofing, which will be much cheaper and more durable than any other metallic roofing now in use.

The proportions of the ingredients are as follows, viz:

Eighty-five (85) parts of pure lead to twelve (12) parts of tin and three (3) parts of copper; or, if a finer quality is desired, take eighty (80) parts of lead to sixteen (16) parts of tin and four (4) parts of copper.

To enable others skilled in the art to make and use my invention, I will proceed to describe the manner in which I usually combine the above-named metals.

The tin is first melted, and the copper then gradually added thereto. When both are fused and intimately mixed, the lead is added to the mixture of copper and tin, and when melted sufficiently, the whole is to be thoroughly mixed by stirring. The melted alloy is then cast in an iron ingot-mould, of the proper form to roll into sheets of the required size and thickness.

Having thus described my invention,

What I claim as new, and desire to secure by Letters Patent, is—

As an article of manufacture, a non-corrosive metallic roofing, composed entirely of tin, copper, and lead, in the proportions substantially as herein set forth.

In testimony that I claim the foregoing, I have hereunto set my hand, this 13th day of March, 1869.

OLIVER T. MAY.

Witnesses:

SAMUEL L. CONDÉ,  
WARREN G. DODGE.